# EUROPEAN PATENT SPECIFICATION

(11) **EP 0 143 782 B1**
(45) Date of publication and mention of the grant of the patent: **24.02.1988**
(21) Application number: 83903622.5
(22) Date of filing: 14.11.1983
(51) Int. Cl.: C10L 1/32

(54) **COAL-WATER DISPERSION**
KOHLE-WASSER-DISPERSION
DISPERSION CHARBON-EAU

(30) Priority: 12.11.1982 WO PCT/EP82/00244; 04.02.1983 WO PCT/SE83/00039; 14.06.1983 SE 8303364
(43) Date of publication of application: 12.06.1985
(73) Proprietor: FLUIDCARBON INTERNATIONAL AB, S-213 75 Malmö (SE)
(72) Inventor: STIGSSON, Lars, Lennart, S-223 61 Lund (SE)
(74) Representative: Ström, Tore
(86) International application number: SE8300396
(87) International publication number: WO8401957

(56) References cited:
- EP-A- 0 077 909
- WO-A-83/04045
- SE-A-81 046 450
- US-A- 4 358 293
- US-A- 4 398 918
- US-A- 4 398 919
- Patent Abstracts of Japan, vol. 5, no. 140 C70
- Patent Abstracts of Japan, vol. 5, no. 156 C 74
- WO A 83/01069

## Description

The present invention relates to a liquid dispersion of pulverized coal, which has a very long storage life and is suitable for transport and energy production.

A dispersion of coal is considerably less polluting and can be more easily handled than solid coal and also eliminates some risks involved in transport and storage. Such a dispersion is also preferred from an economical point of view.

The reason for using coal dispersions is the planned increased use of coal as a basic energy source in large as well as small plants for producing electricity and heat. The handling of solid coal in this connection is difficult for several reasons and, therefore, the transformation of the coal to liquid form generally is considered an interesting method. Chemical conversion of coal to a liquid product, so-called liquefaction, still cannot compete with oil and it is considered that this method can contribute to the global energy provision only marginally before the year 2000. Chemical conversion of the coal to a gaseous product, so-called gasification, seems to be a more prosperous method of utilizing coal. However, also this method still involves considerable technical difficulties although large resources have been spent on technical development.

Physical conversion is another method of transforming the coal into liquid form, and the invention relates to this method. It is practised by dispersion in a liquid which may consist of water only or water in combination with some organic fuel such as heating oil, methanol, etc.

The dispersion of the invention contains water, additives and pulverized coal, the surface of which has been modified by adsorption of zwitterionic or other hydrophobizing substances, the coal content being at least 55% by weight of the dispersion, at least one of the additives included in the dispersion being a water-soluble ionic surfactant polymer having a mole weight over 1500 and containing at least one hydrophobic part with affinity to the coal surface, and at least one water-soluble part based on ethylene oxide with the mole weight exceeding 1,000.

One of the problems in producing a coal-water fuel is that the surface structure of the coal is modified in removing impurities, often by means of chemical additives, and that the dispersion of the coal particles in a later processing stage will be more difficult as a consequence thereof.

WO 83/00500 makes reference to the addition of anionic surfactants to surface modified coal, and WO 83/04045 discloses in general the use of non-ionics and cationic, anionic or zwitterionic additives to coal which may be subjected to preliminary hydrophobating treating.

According to the invention the dispersion of the kind referred to above has obtained the characterizing features defined in any of claims 1, 3 and 6.

When coal-water dispersions which by definition are thermodynamically instable, are being stabilized the sedimentation and aggregation rates are reduced, in applying the invention, by creating a barrier which counteracts the particle attraction. This repulsive effect can be achieved by three main principles: electrostatic stabilization, sterical stabilization, and stabilization by means of hydration forces. The stabilization changes the energy of the particles and/or creates a high barrier preventing particle attraction. On the basis of these principles it is possible to stabilize high contents of coal particles in a water solution by the addition of small amounts of organic additives.

In order to create new colloidal systems it is necessary to impart to the system such properties that the attraction forces between the particles are minimized and a repulsive barrier against flocculation and subsequent sedimentation is developed. Some form of sterical stabilization by means of hydrophilic polymers provides favourable conditions for a long-term stabilization of coal-water dispersions.

The process of manufacturing a coal-water fuel often includes removal of inorganic constituents in one way or the other.

Initially, the coal is ground in one or more mills to a polydisperse particle size distribution. All particles are smaller than about 300 microns and about 35% of the total amount are smaller than 40 microns.

When manufacturing a coal-water fuel according to the present invention, a main process step included therein is a flotation enrichment of the coal, which by selective hydrophobization and charging separates coal and contaminants. For this purpose, different types of reagents are used which generally comprise mixtures of aliphatic alcohols together with a frothing agent. Other reagents which are suitable in the flotation of coal are mixtures of zwitterionic surfactants and oils insoluble in water together with a frothing agent and trace amounts of alkylsulpho-succinates.

After the flotation process the coal is dewatered mechanically, e.g. by means of a rotating vacuum filter. The use of surface-active substances in dewatering coal has been studied in laboratories as well as pilot scale. It has been found that there are two types of surfactants improving the degree of dewatering:
1) Surfactants changing the surface tension of the water.
2) Substances having hydrophobizing properties.

Among surfactants of the first main type anionic surfactants have shown to be the most suitable. Examples of surfactants which can be used are alkylaryl-sulphonates and alkylsulpho-succinates.

In the final processing stage in manufacturing the coal-water fuel a dispersion agent and possibly a stabilizer are added. Among dispersion agents already known for pulverized coal in water or oil are e.g: anionic polynaphthalene sulphonates, polycarboxylic acids and non-ionic ethylene oxide derivatives.

It is previously known that the total amount of dispersion agent calculated as a weight percentage of the total dispersion, is completely decisive for the physical properties of the dispersion. Apart from the coal, the dispersion agent is one of the significant items of expenditure in the manufacture of the dispersion.

It has also been found that different types of coal require different types of dispersion agents and therefore the present invention provides a method of effecting dispersion of coal particles with the same type of basic compound but with different charges. Particularly active dispersion agents are built-up around a hydrophobic aromatic part and one or more hydrophilic ethylene oxide chains.

The molecular charge can be anionic, cationic or preferably zwitterionic. The charge of the molecule is varied with the surface charge of the coal itself.

Among the zwitterionic compounds of this type it is suitable to choose a zwitterionic alkylaryl ethoxylate e.g. sodium nonyl phenetoxy methyl tauride. The compound is most easily produced by a reaction between the terminal hydroxide group of the nonyl phenol ethoxylate and sulphonyl chloride, the resultant halide being allowed to react with sodium methyl tauride.

The sum formula of the compound is

Other zwitterionic compounds which constitute excellent dispersion media for certain coals are the zwitterionic salts of ethoxylated quaternary nitrogen compounds, e.g. the sulphates. This type of compound is sold commercially by GAF under the designation PC-37.

Cationic compounds which can be used according to the invention are based primarily on pyridine and quinoline. An aromatic ring structure with hydrophobic properties is common to them all. Pyridine reacts with ethers to form compounds of the type alkoxymethyl pyridine. These cationic dispersion agents, moreover, are characterized in that they contain at least 50 ethylene oxide units. They may also be based on isoquinoline, benzindiazole, benzthiazole, benztriazole, pyrrolidine, imidazole, piperidine, morpholine or their derivatives.

The anionic dispersion agents, which are applied to a lesser extent due to the higher price thereof, are salts of alkylaryl oxyethylene oxyalcohols, e.g. an ammonium salt of an alkyl phenoxy polyethylene oxyethanol. Anionic compounds of this type are most appropriate for hydrophilic coals.

All dispersion agents according to the invention have mole weights over 1,500 and are soluble in water.

The invention will be described by means of an illustrative example.
1) A non-micelle-forming and therefore relatively sparingly soluble zwitterionic surfactant such as lecithin or alkyl betaine, is emulsified in water to form a liquid crystalline phase. The emulsion (0.03% by weight of the coal) is supplied to the grinding step of the fuel preparation process. In a mixing step immediately before the flotation step, a preparation consisting of lecithin, hexadecane and methylisobutyl ketone is added in the ratio 1/5/2. The total additive amount and the composition can be varied for different coal qualities (0.01-0.05% by weight of the coal). After the flotation process, a small amount of alkylsulpho-succinate (10-50 g/ton coal) is added to improve the dewatering degree in the filter. The filter cake contains between 15 and 22% moisture.
2) About 90 grammes of the moist purified coal filter cake from the process (22.2%) is homogenized and mixed with 0.25 grammes dispersion agent dissolved in water and comprising an ammonium salt of nonyl phenoxy polyethylene oxyethanol with a mole weight of about 5,000.

By varying the concentration of the aqueous solution with regard to the dispersion medium the resultant coal content of the mixture is adjusted to 70%. The dispersion obtained in this manner has excellent properties for transport and direct combustion as a liquid fuel.

In order to achieve storage stability, stability against coalescense and sedimentation a gelation agent can be added to the dispersion. The gelation can be reversible as well as irreversible. Reversible gelation can be attained with small amounts of polysaccharide, xantan gum, guar-gum, alginate or a modified starch in combination with a metal ion, e.g. aluminium or boron. The reversible gelation process can be controlled by changing the temperature or the pH.

Irreversible gelation of the coal-water dispersion can be effected e.g. by means of different clays, bentonite, Chinese clay, etc. The fuel product obtained has now a clearly pseudoplastic rheology.

The coal-water fuel has been found to be a very good oil substitute for heat as well as steam production. The fuel is purified from a lot of inorganic contaminants and is preferred from an environmental and handling point of view to conventional coal technology.

## Claims

1. Dispersion containing water, additives and pulverized coal, the surface of which has been modified by adsorption of zwitterionic or other hydrophobizing substances, the coal content being at least 55% by weight of the dispersion, at least one of the additives included in the dispersion being a water-soluble ionic surfactant polymer having a mole weight over 1500 and containing at least one hydrophobic part with affinity to the coal surface, and at least one water-soluble part based on ethylene oxide with the mole weight exceeding 1,000, characterized in that the additive, having zwitterionic charge, contains zwitterionic groups of imidazolene derivatives, betaine derivatives, zwitterionic amino acid derivatives, or lecithin derivatives.

2. Dispersion as claimed in claim 1, characterized in that the additive is a zwitterionic salt of an ethoxylated quaternary nitrogen compound or a zwitterionic alkylaryl ethoxylate.

3. Dispersion containing water, additives and pulverized coal, the surface of which has been modified by adsorption of zwitterionic or other hydrophobizing substances, the coal content being at least 55% by weight of the dispersion, at least one of the additives included in the dispersion being a water-soluble ionic surfactant polymer having a mole weight over 1500 and containing at least one hydrophobic part with affinity to the coal surface, and at least one water-soluble part based on ethylene oxide with the mole weight exceeding 1,000, characterized in that the hydrophobic part is built-up on one or more aromatic groups and that the additive, having cationic charge, is an ethoxylated cyclic alkylammonium compound.

4. Dispersion as claimed in claim 3, characterized in that the additive is based on an unsaturated heterocyclic compound including at least one of the groups pyridine, quinoline, isoquinoline, benzindiazole, benzthiazole, benztriazole, pyrrolidine, imidazole, or derivatives of these groups.

5. Dispersion as claimed in claim 3, characterized in that the additive is based on a saturated nitrogen compound including at least one of the groups piperidine, morpholine or derivatives thereof.

6. Dispersion containing water, additives and pulverized coal, the surface of which has been modified by adsorption of zwitterionic or other hydrophobizing substances, the coal content being at least 55% by weight of the dispersion, at least one of the additives included in the dispersion being a water-soluble ionic surfactant polymer having a mole weight over 1500 and containing at least one hydrophobic part with affinity to the coal surface, and at least one water-soluble part based on ethylene oxide with the mole weight exceeding 1,000, characterized in that the hydrophobic part is built-up on one or more aromatic groups and that the additive, having anionic charge, is a salt of an alkylaryl oxyethylene oxyalcohol.

7. Dispersion as claimed in claim 6, characterized in that the additive is an ammonium salt of an alkyl phenoxy polyethylene oxyethanol.

## Patentansprüche

1. Dispersion, die Wasser, Additive und pulverisierte Kohle enthält, deren Oberfläche durch Adsorption zwitterionischer oder anderer hydrophobierender Substanzen modifiziert wurde, wobei der Kohlegehalt mindestens 55 Gew.-% der Dispersion beträgt, zumindest eines der in der Dispersion enthaltenen Additive ein wasserlösliches ionisches oberflächenaktives Polymer ist, das ein Molekulargewicht von über 1500 aufweist und zumindest einen hydrophoben Teil mit Affinität gegenüber der Kohleoberfläche und mindestens einen wasserlöslichen Teil enthält, der auf Ethylenoxid basiert, wobei das Molekulargewicht 1000 überschreitet, dadurch gekennzeichnet, daß das Additiv mit zwitterionischer Ladung zwitterionische Gruppen von Imidazolinderivaten, Betainderivaten, zwitterionischen Aminosäurederivaten oder Lecithinderivaten enthält.

2. Dispersion nach Anspruch 1, dadurch gekennzeichnet, daß das Additiv ein zwitterionisches Salz einer ethoxilierten quaternären Stickstoffverbindung oder ein zwitterionisches Alkylarylethoxilat ist.

3. Dispersion, die Wasser, Additive und pulverisierte Kohle enthält, deren Oberfläche durch Adsorption zwitterionischer oder anderer hydrophobierender Substanzen modifiziert wurde, wobei der Kohlegehalt mindestens 55 Gew.-% der Dispersion beträgt, zumindest eines der in der Dispersion enthaltenen Additive ein wasserlösliches ionisches oberflächenaktives Polymer ist, das ein Molekulargewicht von über 1500 aufweist und mindestens einen hydrophoben Teil mit Affinität gegenüber der Kohleoberfläche und mindestens einen wasserlöslichen Teil enthält, der auf Ethylenoxid basiert, wobei das Molekulargewicht 1000 überschreitet, dadurch gekennzeichnet, daß der hydrophobe Teil auf einer oder mehreren aromatischen Gruppen aufgebaut ist, und daß das Additiv mit kationischer Ladung eine ethoxilierte zyklische Alkylammoniumverbindung ist.

4. Dispersion nach Anspruch 3, dadurch gekennzeichnet, daß das Additiv auf einer ungesättigten heterozyklischen Verbindung basiert, die zumindeste eine der Gruppen von Pyridin, Chinolin, Isochinolin, Benzindiazol, Benzthiazol, Benztriazol, Pyrrolidin, Imidazol oder Derivate dieser Gruppen enthält.

5. Dispersion nach Anspruch 3, dadurch gekennzeichnet, daß das Additiv auf einer gesättigten Stickstoffverbindung basiert, die zumindest eine der Gruppen von Piperidin, Morpholin oder Derivate davon enthält.

6. Dispersion, die Wasser, Additive und pulverisierte Kohle enthält, deren Oberfläche durch Adsorption zwitterionischer oder anderer hydrophobierender Substanzen modifiziert wurde, wobei der Kohlegehalt mindestens 55 Gew.-% der Dispersion beträgt, zumindest eines der in der Dispersion enthaltenen Additive ein wasserlösliches ionisches oberflächenaktives Polymer ist, das ein Molekulargewicht von über 1500 aufweist und zumindest einen hydrophoben Teil mit Affinität gegenüber der Kohleoberfläche und mindestens einen wasserlöslichen Teil enthält, der auf Ethylenoxid basiert, wobei das Molekulargewicht 1000 übersteigt, dadurch gekennzeichnet, daß der hydrophobe Teil auf einer oder mehreren aromatischen Gruppen aufgebaut ist und daß das Additiv mit anionischer Ladung ein Salz eines Alkylaryloxiethylenoxialkohols ist.

7. Dispersion nach Anspruch 6, dadurch gekennzeichnet, daß das Additiv ein Ammoniumsalz von Alkylphenoxipolyethylenoxiethanol ist.

## Revendications

1. Dispersion contenant de l'eau, des additifs et du charbon pulvérisé dont la surface a été modifiée par adsorption de substances zwitterioniques ou autres substances conférant le caractère hydrophobe, la teneur en charbon étant d'au moins 55% en poids de la dispersion, au moins l'un des additifs inclus dans la dispersion étant un polymère surfactant ionique hydrosoluble de poids moléculaire supérieur à 1500 et contenant au moins une partie hydrophobe douée d'affinité pour la surface du charbon, et au moins une partie hydrosoluble à base d'oxyde d'éthylène de poids moléculaire dépassant 1000, caractérisée en ce que l'additif à charge zwitterionique contient des groupes zwitterioniques de dérivés d'imidazolène, de dérivés de bétaïne, de dérivés zwitterioniques d'amino-acides ou de dérivés de lécithine.

2. Dispersion suivant la revendication 1, caractérisée en ce que l'additif est un sel zwitterionique d'un composé d'azote quaternaire éthoxylé ou un éthoxylate d'alkylaryle zwitterionique.

3. Dispersion contenant de l'eau, des additifs et du charbon pulvérisé dont la surface a été modifiée par adsorption de substances zwitterioniques ou d'autres substances conférant le caractère hydrophobe, la teneur en charbon étant d'au moins 55% en poids de la dispersion, au moins l'un des additifs inclus dans la dispersion étant un polymère surfactant ionique hydrosoluble ayant un poids moléculaire supérieur à 1500 et contenant au moins une partie hydrophobe douée d'affinité pour la surface du charbon, et au moins une partie hydrosoluble à base d'oxyde d'éthylène de poids moléculaire dépassant 1000, caractérisée en ce que la partie hydrophobe est édifiée sur un ou plusieurs groupes aromatiques et en ce que l'additif à charge cationique est un composé d'alkylammonium cyclique éthoxylé.

4. Dispersion suivant la revendication 3, caractérisée en ce que l'additif est à base d'un composé hétérocyclique non saturé comprenant au moins l'un des groupes pyridine, quinoléine, isoquinoléine, benzodiazole, benzothiazole, benzotriazole, pyrrolidine, imidazole ou des dérivés de ces groupes.

5. Dispersion suivant la revendication 3, caractérisée en ce que l'additif est à base d'un composé azoté saturé comprenant au moins l'un des groupes pipéridine, morpholine ou leurs dérivés.

6. Dispersion contenant de l'eau, des additifs et du charbon pulvérisé dont la surface a été modifiée par adsorption de substances zwitterioniques ou autres substances conférant le caractère hydrophobe, la teneur en charbon étant d'au moins 55% en poids de la dispersion, au moins l'un des additifs inclus dans la dispersion étant un polymère surfactant ionique hydrosoluble ayant un poids moléculaire supérieure à 1500 et contenant au moins une partie hydrophobe douée d'affinité pour la surface du charbon, et au moins une partie hydrosoluble à base d'oxyde d'éthylène de poids moléculaire depassant 1000, caractérisée en ce que la partie hydrophobe est édifiée sur un ou plusieurs groupes aromatiques et en ce que l'additif à charge anionique est un sel d'un oxyalcool oxyéthylénique alkylarylique.

7. Dispersion suivant la revendication 6, caractérisée en ce que l'additif est un sel d'ammonium d'un alkylphénoxypolyéthylène-oxyéthanol.
